

Sept. 3, 1968

R. C. KNOWLTON

3,399,439

PROCESS FOR CRIMPING ABRASIVE FIBERS

Filed Jan. 24, 1967

FIG. 1



FIG. 2



FIG. 3



FIG. 4



INVENTOR  
ROBERT C. KNOWLTON

BY *Morris E. Beckman*  
ATTORNEY

## 1

3,399,439

**PROCESS FOR CRIMPING ABRASIVE FIBERS**  
 Robert C. Knowlton, Kinston, N.C., assignor to E. I. du  
 Pont de Nemours and Company, Wilmington, Del., a  
 corporation of Delaware

Filed Jan. 24, 1967, Ser. No. 611,385  
 4 Claims. (Cl. 28—72)

**ABSTRACT OF THE DISCLOSURE**

The improvement in the process of crimping synthetic filamentary tows which are abrasive to metals while in high pressure rubbing contact therewith in a stuffer-box type crimpler. The improvement comprising blending from 5% to 55% of a non-abrasive fiber with the abrasive fiber prior to crimping and guiding the blend components through the stuffer-box crimpler in such a manner as will provide a shield of the relatively non-abrasive fiber between the abrasive fiber and the stationary portions of the crimping apparatus that contact the moving tow thereby reducing wear and the attendant fiber damage.

**BACKGROUND OF THE INVENTION***Field of the invention*

This invention relates to stuffer-box crimping of synthetic filamentary tows and more particularly to an improved process for crimping of tows which are abrasive under high-pressure rubbing contact with metals.

*Description of the prior art*

It is well-known to crimp synthetic filamentary tows in apparatus comprising a set of advancing rolls which force the tow into a channel the egress from which is blocked by a gate urged toward the closed position by one of a variety of means. Such crimping apparatus is described in the Hitt U.S. Patent 2,747,233 which issued May 29, 1956, for example. In these crimpers, the advancing rolls are yieldably loaded toward each other to permit the slight opening and closing motion required to accommodate the unavoidable slight variations in thickness of the tow in their nip due to position-to-position migration of individual filaments over preceding guides. The filaments are prevented from spreading beyond the ends of the rolls by the presence of disc shaped inserts which are held firmly against the rolls at each end of the nip.

It has been found that certain types of filamentary tows may not continuously be processed to crimped tows of good quality in stuffer-box crimpers known to the art. Products which tend to abrade metals under rubbing, high-pressure contact will rapidly wear the discs to form a depression with sharp edges therein. The tow is severely damaged by contact with such worn discs thereby necessitating frequent process interruptions for disc replacement to avoid an unacceptable level of filament breaks at the edges of the tow.

Products which tend to abrade metals include those fibers classified as "dull" in luster due to the presence of a rather large amount of delustering (opacifying) pigment such as titania and also those fibers which have an intentionally roughened surface resulting from the incorporation of other particulate matter that may be larger in size and smaller in quantity than the titania delustrant. The dull products provide improved "cover" (opacity) in fabrics constructed from them and the roughened fiber finds a variety of uses where a lower fiber-to-fiber friction is desirable.

Rosenstein et al. U.S. Patent 3,164,882, which issued Jan. 12, 1965, teaches the use of an endless cushion apron

## 2

or limp flexible sheathing which is made of a filament sliver, knitted or woven webbing or such like material of a durable and pliable nature for protecting the filaments being crimped as they pass between the pressing means within the stuffer-box type crimpler. Rosenstein et al. among other things, is concerned with crimping fibers which heretofore could not be crimped because of their inability to withstand stresses or strains exerted transversely of their longitudinal axis. The present invention concerns the improvement in the process of crimping fibers that are abrasive to metals and the reduction of the attendant fiber damage from rubbing the otherwise abraded metal parts of the crimpler. The present invention also accomplishes its purpose without reduction in crimpler capacity. In the present invention the shielding fiber (low-abrasive) is part of the production being crimped whereas in Rosenstein the endless sheathings are in essence being crimped but are not part of the crimpler production, thereby decreasing the crimpler efficiency.

Rosenstein teaches nothing about the abrasiveness of the sheathing as compared to the abrasiveness of the production being crimped.

Though the process of Rosenstein et al. may lessen fiber damage caused by high pressure rubbing contact of the fiber against the stationary metal parts of the crimpler it does not accomplish this goal in a manner analogous to that of the present invention. Rosenstein lessens the damage by advancing the cushion sheathing simultaneously with the production filaments being crimped, thereby preventing high pressure rubbing contact between the faces of the production rope and the crimpler. The present invention accomplishes its purpose without eliminating high pressure rubbing contact between production and the crimpler as in Rosenstein et al. at the expense of crimpler efficiency, but accomplishes its purpose by the critical selection of shield fibers designed to be compatible with the highly abrasive fiber in textile fabrics prepared from them and to be relatively low in abrasion of metal while in high pressure rubbing contact therewith.

A process for stuffer-box crimping of abrasive fibers without the attendant fiber damage is highly desirable.

**SUMMARY**

This invention provides an improved process for crimping fibers that are abrasive to metals.

This and other advantages are provided by this improvement invention in the process for crimping fibers which are abrasive to metals which comprises blending from 5% to 55%, preferably 10% to 25% of a low abrasive fiber with the abrasive fibers prior to crimping and guiding the blend components to the stuffing-rolls nip in such a manner as will provide a shield of relatively non-abrasive fiber between the abrasive fiber and the crimpler discs which are inserted adjacent the nip of the stuffing rolls to hold the tow within the nip and to guide the tow into the crimpler. The non-abrasive filaments may be any of the class of fibers which are relatively low in disc-wear rate, but it generally will be preferable to choose as the shield fiber one which otherwise resembles the predominant fiber in physical and chemical properties as closely as possible. In this manner, the presence of the shield as a diluent will have little or no effect on the characteristics of the products made therefrom. It will be recognized, however, that to attain certain novel or special effects it may be desirable to employ as a shield fiber one which has distinctly different characteristics.

Subsequent to crimping, the tow may be handled in a variety of ways depending on its intended utility. If cut to staple, the two types of fiber will be intimately blended by subsequent processing to useful structures. If finished as tow for textile processing on one of the tow-breaking

means, blending of the two fiber components will be accomplished in the early stages of the series of subsequent operations associated with this system.

#### BRIEF DESCRIPTION OF THE DRAWING

FIGURE 1 is a diagrammatic sketch of a stuffer box type crimper that is useful in carrying out the process of this invention. The tow to be crimped is indicated by 5 and the driven feed rolls are indicated by numerals 6 and 7.

FIGURE 2 is a view taken on line 2—2 of FIGURE 1 to illustrate the improvement feature in the crimping process of this invention which is the reduction of the frictional wear of the inserts 8 and 9 and reduction of the resulting fiber and tow damage caused by high pressure rubbing contact of the edges of the tow 5 with the inserts.

FIGURE 3 is a view of the tow prior to crimping taken across the tow width with the semidull (low abrasive) edges indicated by 10

FIGURE 4 is a view taken across the tow width after crimping with the semidull (low abrasive) edges indicated by 10.

A more complete description of the stuffing box type crimper useful in carrying out the process of this invention may be had by reference to Hitt, U.S. Patent 2,311,174, which issued Feb. 16, 1943, and to Hitt, U.S. Patent 2,747,233, which issued May 29, 1956.

This invention is further illustrated by the following example.

#### EXAMPLE

A total of 46 bobbins of 600-filament, 1.5 denier-per-filament drawn polyester yarn is crimped in a stuffing-box crimper. Forty-two of the bobbins are dull in luster due to presence of 2.0%  $TiO_2$  delustrant; four bobbins contain semidull yarn which has 0.3%  $TiO_2$ . Two of the semidull yarn ends are guided in such a manner as to lie predominantly at the back side of the bundle as it is guided to the crimper thereby serving as a shield between the dull tow and the back side of the crimper. The remaining two semidull ends are blended with the 42 dull yarns nearer the front side of the bundle. The following table summarizes the results obtained, including a comparison test involving only semidull yarn.

TABLE

| Test   | Percent $TiO_2$ overall | Percent semidull/percent dull | Depth of disc abrasion (microns) |      | Running time (min.) |
|--------|-------------------------|-------------------------------|----------------------------------|------|---------------------|
|        |                         |                               | Front                            | Back |                     |
| A----- | 0.3                     | 100/0                         | 32                               | 49   | 105                 |
| B----- | 1.83                    | 10/90                         | 81                               | 24   | 90                  |
| C----- | 1.83                    | 10/90                         | 151                              | 15   | 45                  |

It will be seen that the presence of semidull fiber adjacent to the crimper disc during crimping of dull fiber substantially reduces the rate of wear, but that the advantages of this invention are best obtained by guiding the shield fiber so as to lie between the abrasive fiber and the discs.

In a second test, in which 24% semidull fiber was equally divided and oriented at both sides of a dull tow, abrasion depth was found to average 65—75 microns after 40 minutes of operation, compared with 150 microns during processing of 100% dull tow.

What is claimed is:

1. In the process of crimping a plurality of continuous filament yarns which are highly abrasive to metal while in high pressure rubbing contact therewith and having opacifying particulate matter in the yarns, the process being of the type including the steps of:
  - (a) continuously bringing together in the form of a rope a plurality of separated yarns;
  - (b) continuously guiding said rope of yarns into the nip of a pair of counter-rotating rotary pressure members;
  - (c) discharging said yarns from said nip into an enclosed housing adapted to accumulate and restrain the yarns, whereby the individual continuous filaments of said yarns are caused to continuously crimp as they are discharged from said nip, the yarns being held within said nip and guided to said housing by means of inserts held firmly against the ends of said nip;
  - (d) releasing the resultant crimped yarns from said housing;
- 20 wherein the improvement comprises
  - (e) continuously guiding on the edges of said rope in step (a) from 5% to 55% based on total rope of low abrasive yarns having a lesser amount of opacifying particulate matter;
  - (f) guiding said low abrasive yarn in step (b) between said high abrasive yarn and said inserts whereby said low abrasive yarn shields the high abrasive yarn from high pressure rubbing contact with said inserts; and then
  - (g) combining said low abrasive yarn with said high abrasive yarn;
- 25 said low abrasive yarn being compatible in textile fabrics with said high abrasive yarn.
- 30 2. The process as in claim 1 wherein said low abrasive yarn in step (e) is from 10% to 25% of the total rope.
3. The process as in claim 1 wherein said high abrasive yarns contain from 1% to about 3% titania pigment ( $TiO_2$ ) and said low abrasive yarns contain from about 0.1% to about 0.5% of titania pigment ( $TiO_2$ ).
4. The process as in claim 3 wherein said high and low abrasive yarns are essentially polyesters.

#### References Cited

#### UNITED STATES PATENTS

1,893,809 1/1933 Stone et al.

#### FOREIGN PATENTS

962,516 7/1964 Great Britain.

LOUIS K. RIMRODT, Primary Examiner.